

# United States Patent

[19]

Walters et al.

[11] 3,849,146

[45] Nov. 19, 1974

[54] DIRECT-PRINT LIGHT-DEVELOPABLE SILVER HALIDE EMULSION CONTAINING CYCLIC DIOXIDE OR SELENONE AS SENSITIZER

[75] Inventors: David W. Walters, Williamson; Robert E. Heeks, Penfield; Donald P. Sullivan, Rochester, all of N.Y.

[73] Assignee: Xerox Corporation, Stamford, Conn.

[22] Filed: Jan. 2, 1973

[21] Appl. No.: 320,422

[52] U.S. Cl..... 96/107, 96/108, 96/109

[51] Int. Cl..... G03c 1/28

[58] Field of Search..... 96/107, 108, 109

[56] References Cited

UNITED STATES PATENTS

3,507,656 4/1970 Sincius..... 96/108  
3,594,172 7/1971 Sincius..... 96/108

3,649,289 3/1972 Hiller ..... 96/107

Primary Examiner—Ronald H. Smith

Assistant Examiner—Won H. Louie, Jr.

Attorney, Agent, or Firm—James J. Ralabate; David C. Petre; George J. Cannon

[57]

## ABSTRACT

A photographic emulsion of the silver halide direct-print light-developable type containing cyclic compounds of the general formula:



wherein X may be S or Se; and hydrogen and lower alkyl substitution products thereof. Optimum results may be obtained by addition of iodide, gold and silver thiocyanate sensitizers.

8 Claims, No Drawings

**DIRECT-PRINT LIGHT-DEVELOPABLE SILVER HALIDE EMULSION CONTAINING CYCLIC DIOXIDE OR SELENONE AS SENSITIZER**

**BACKGROUND OF THE INVENTION**

This invention relates in general to photographic emulsions. More specifically, the invention concerns photographic emulsions of the "direct-print light-developable" type.

The term "direct-print light-developable" refers to layers, generally deposited on a film or paper substrate, containing photosensitive materials upon which a visible image is obtained after an initial exposure to a pattern of high intensity light or other electromagnetic radiation has been utilized to form a latent image; the visible image being obtained by additional overall exposure to generally lower intensity radiation. This additional exposure is known as "latensification." The entire sheet surface is exposed including exposure of the background area and re-exposure of the area upon which the initial image was formed. Direct-print light-developable materials are distinguished from developing-out emulsions in that they do not require a wet development treatment, such as a multi-step chemical development after initial exposure to produce a visible image. While the direct-print light-developable materials of this invention may be used for ordinary photographic purposes, they are particularly sensitive to a high intensity beam of light or other electromagnetic radiation and are, therefore, especially useful in high speed recording such as oscillographic recording and the like.

Direct-print light-developable type materials are today in general use for recording of oscillographic traces. However, the direct-print light-developable materials of the prior art are not entirely satisfactory for this recording purpose for a number of reasons. For example, it is generally true that the prior art materials which exhibit high sensitivity to an exposure of short duration to a high intensity beam tend to exhibit a correspondingly low degree of background stability. The latensification procedure for these materials is highly critical and accordingly is exceedingly difficult to carry out. The latent image may be entirely lost during the latensification operation where the background darkens too rapidly. In other cases, a phenomenon known as "reversal" may occur, this being a darkening of the background which proceeds at a more rapid rate than darkening of the image trace. In these situations, the trace may be temporarily or permanently obscured. Conversely, materials which exhibit a high degree of background stability tend to exhibit a correspondingly low degree of sensitivity to the recording beam and, thus, the minimum exposure time is far above that desired for use in modern recording instruments.

Sensitized direct-print light-developable materials have been described utilizing the sensitization of silver halide emulsions with a combination of a plumbous salt and a thiourea, thiosemicarbazide or mercapto succinic acid. While this material shows increased sensitivity, it is not as stable when exposed for prolonged times to daylight or normal room lighting as would be desirable. Upon prolonged exposure to ordinary illumination, the background darkens and the image regresses depending upon the viewing conditions which reduces the ratio between background and image density.

On occasion it is desirable to make a truly permanent record of an oscillographic trace. In this circumstance, it is desirable to develop the usual direct-print light-developable emulsion either before or after latensification by chemical developing-out techniques. Many conventional direct-print light-developable emulsions require special developing materials and procedures. Preferably, a direct-print light-developable emulsion used in an oscillographic recorder should be developable by the usual direct-print light-developable techniques or alternatively, by means of a chemical developing-out process.

Different direct-print light-developable materials produce image traces and background areas of varying colors. Typically, the image trace may be developed as a brown or blue-grey line. The background areas which would preferably remain white often acquire a uniform color, typically, pink, brown or blue. Preferably, there should be good contrast between the trace and backgrounds both in density and in color to permit convenient and accurate examination and evaluation of the trace.

It is also desirable to have access to the information recorded on the material as rapidly as possible. The access time is the period of time which elapses between the imagewise exposure and the first appearance of the recorded information in response to latensification.

Thus, there is a continuing need for improved direct-print light-developable materials having improved sensitivity, stability and appearance characteristics.

**SUMMARY OF THE INVENTION**

It is, therefore, an object of this invention to provide a direct-print light-developable emulsion overcoming the above-noted disadvantages.

Another object of this invention is to provide a novel light sensitive composition.

Another object of this invention is to provide a more sensitive dry process for the reproduction of images.

Still another object of this invention is to provide a photosensitive emulsion which may be developed either by direct-print light-developable techniques or by chemical developing-out techniques.

Still another object of this invention is to provide an improved direct-print light-developable emulsion which possesses both a high degree of photosensitivity and a high degree of background stability under general latensification.

Another object of this invention is to provide a photosensitive emulsion which provides relatively improved access time.

A still further object of this invention is to provide a direct-print light-developable emulsion resistant to light degradation after imaging.

A further object of this invention is to provide a direct-print light-developable emulsion which is capable of producing images having improved contrast and color characteristics.

The above objects and others are accomplished in accordance with this invention by providing a photographic direct-print light-developable emulsion comprising a photosensitive silver halide and gelatin containing cyclic compounds of the general formula:



wherein X may be S or Se; and hydrogen and lower alkyl substitution products thereof as a sensitizer. Preferably, the emulsions also contain iodide, gold and silver thiocyanate.

Good results have been obtained using from about 0.02 to 20.0 mole percent of cyclic compounds of the formula given above based on moles of silver in the silver halide grains. Approximately 0.01 to 25 mole percent iodide is added to the emulsion. Additional benefits primarily in reduced access time and increased image contrast results from the addition of from about 0.001 to about 1.0 mole percent gold to emulsions containing compounds within the formula given below. Optimum results are obtained with the addition of from about 0.1 to 25 mole percent silver thiocyanate based on the silver in the silver halide grains. The use of silver thiocyanate is disclosed in our copending application Ser. No. 125,816, filed Mar. 18, 1971 the disclosure of which is incorporated herein by reference. The sensitizers may be added in any suitable form. The silver thiocyanate is added in the form of a gel suspension. Typically, gold and iodide are added as water soluble complexes or salts in water. However, this is not necessary. For example, some ingredients may be added as solids or in other solvents such as acids, bases or water miscible organic solvents.

As is further pointed out in the Examples below, the use of iodide alone provides images having low contrast and low sensitivity. The addition of compounds of the general formula to the emulsion containing iodide improves contrast; that is, the difference in density between the image area  $D_{max}$  and the density of the background areas  $D_{min}$  is greater. The difference between  $D_{max}$  and  $D_{min}$  is known as  $\Delta D$ . It also improves sensitivity which increases the speed at which images may be recorded. Further, the addition of gold to the emulsions containing cyclic compounds of the general formula given above and iodide improves the access time. Optimum image quality is achieved by adding silver thiocyanate.

The emulsion layer may comprise any suitable conventional silver halide and binder. Best results have been obtained with silver chlorobromide emulsions these are, therefore preferred. These emulsions are made by first forming silver chloride and then converting substantially all of the silver chloride into a mixed crystal of predominantly silver bromide by adding a soluble bromide salt to the emulsion. Gelatin is the conventional binder for photographic emulsions. However, any other suitable binder, such as polyvinylalcohol, may be used if desired. Ordinarily, this layer should be no greater than about 25 microns in thickness. For optimum results, the layers should contain about three grams of elemental silver per square meter of coated emulsion. The emulsion layer may contain additional ingredients to enhance, synergize or otherwise modify its characteristics, as desired. Typical silver bromide emulsions are described in "Photographic Emulsions," E. J. Wall, American Photographic Publishing Co., Boston (1929) and in U.S. Pat. No. 3,249,440.

Silver thiocyanate is added to the emulsion in the form of a suspension, preferably about 0.6 mole AgCNS per liter of a gelatin suspension. The suspension is formed by adding silver nitrate to potassium thiocyanate in water. The precipitate is dispersed in a gelatin binder. Since the silver thiocyanate formed is light

sensitive, the precipitation and subsequent process steps should be carried out under safelight conditions. The silver thiocyanate is added after the silver halide grains have been formed.

The iodide may be added in the form of any compound which will furnish iodide ions to the suspension and may be water soluble or insoluble. Typical compounds include lead iodide, silver iodide, alkali metal iodides, ammonium iodide, calcium iodide and barium iodide.

The gold may be added in the form of water soluble compounds such as ammonium aurothiocyanate, potassium aurothiocyanate, sodium aurothiocyanate, aurous thiosulfates, alkali metal aurous sulfates, chlorauric acid and alkali metal halides complexed with auric trihalides.

The iodide and gold are also added after the silver halide grains are formed. It is believed therefore that the sensitizers are primarily present on the surface of

20 the silver halide grains. It is also believed that whether the gold is added to the emulsion in the auric or the aurous form that it is converted to or remains aurous because of the presence of thiocyanate. The sensitizers within the general formula given above are also added after the silver halide grain has been formed. The sensitizers are added along with the iodide, bromide and the gold. Preferred compounds within the general formula include: tetrahydrothiophene-1,1-dioxide; 2,5-dihydrothiophene-1, 1-dioxide; 3-methyltetrahydrothiophene-1,1-dioxide and 3-methyl-2, 5-dihydrothiophene-1,1-dioxide.

#### DESCRIPTION OF PREFERRED EMBODIMENTS

The following Examples in the Table further specifically define the present invention with respect to particular sensitizers and the amounts thereof used in the direct-print light-developable emulsions of this invention. All percentages used are mole percent per mole of silver in the silver halide grains unless otherwise indicated. The Examples below utilizing sensitizers within the ranges described above are intended to illustrate various preferred embodiments of the direct-print light-developable emulsions of the present invention.

45 A gelatino-silver halide emulsion for use in the following Examples with different amounts of different sensitizers is prepared as follows: An aqueous solution of silver nitrate is added to an aqueous gelatin solution of potassium chloride in such a manner that there is about 105 mole percent of chloride ion based on the silver nitrate. The resulting mixture is ripened for about 30 minutes at about 160°F. Potassium bromide in an amount sufficient to provide about 120 mole percent based on silver is then added. Ripening is continued for an additional 10 minutes.

55 The emulsion is then chilled, set, shredded and washed to remove excess salts. This material is then melted at about 100°F., the sensitizers to be tested are then added and the mixture is ripened further. Before coating, an additional about 15 mole percent cadmium bromide is added. The emulsion is then coated onto a substrate to obtain a layer having about three grams of elemental silver per square meter.

The direct-print light-developable emulsions thus produced in each Example are tested by exposing in an Edgerton, Germeshausen and Grier Mark VII Sensitometer at 100 microseconds exposure time. The test

strips are exposed through a  $\sqrt{2}$  stepwedge. After exposure the test strips are latensified for about 10 minutes under General Electric Cool White Fluorescent lamps at an illuminational level of about 50 foot candles.

emulsion layer to synergize, enhance or otherwise modify its properties. For example, sensitizing dyes, various finishing aids such as formaldehyde, surfactants, surface active agents such as saponin, humectants such as glycerin, stabilizers such as 7-hydroxy-5-methyl-1,3,4-

TABLE

EXAMPLE NO.

|      | 1<br>Tetrahydro-<br>thiophene-1,<br>1-dioxide          | 2<br>[AgSCN] | 3<br>[AuSCN] | 4<br>[I] | 5<br>Access Time<br>Seconds | 6<br>$\Delta D$ |
|------|--------------------------------------------------------|--------------|--------------|----------|-----------------------------|-----------------|
| I    | 0.00                                                   | 0.00         | 0.00         | 5.60     | 5                           | 0.21            |
| II   | 0.0198                                                 | 0.00         | 0.00         | 5.60     | 7                           | 0.22            |
| III  | 0.198                                                  | 0.00         | 0.00         | 5.60     | 10                          | 0.24            |
| IV   | 1.98                                                   | 0.00         | 0.00         | 5.60     | 8                           | 0.31            |
| V    | 19.8                                                   | 0.00         | 0.00         | 5.60     | 9                           | 0.20            |
| VI   | 0.00                                                   | 8.0          | 0.03         | 5.60     | 6                           | 0.22            |
| VII  | 0.0198                                                 | 8.0          | 0.03         | 5.60     | 4                           | 0.22            |
| VIII | 0.198                                                  | 8.0          | 0.03         | 5.60     | 4                           | 0.32            |
| IX   | 1.98                                                   | 8.0          | 0.03         | 5.60     | 5                           | 0.36            |
| X    | 19.8                                                   | 8.0          | 0.03         | 5.60     | >3                          | 0.26            |
| XI   | 2,5-dihydro-<br>thiophene-1,<br>1-dioxide              | [AgSCN]      | [AuSCN]      | [I]      | Access Time<br>Seconds      | $\Delta D$      |
|      | 1.98                                                   | 8.0          | 0.03         | 5.60     | 4                           | 0.34            |
|      | 3-methyl-<br>tetrahydro-<br>thiophene-1,<br>1-dioxide  | [AgSCN]      | [AuSCN]      | [I]      | Access Time<br>Seconds      | $\Delta D$      |
| XII  | 1.98                                                   | 8.0          | 0.03         | 5.60     | 6                           | 0.31            |
|      | 3-methyl-2,<br>5-dihydro-<br>thiophene-1,<br>1-dioxide | [AgSCN]      | [AuSCN]      | [I]      | Access Time<br>Seconds      | $\Delta D$      |
| XIII | 1.98                                                   | 8.0          | 0.03         | 5.60     | 4                           | 0.37            |

As indicated by the above table, outstanding results are obtained with a direct-print light-developable emulsion sensitized with the sensitizing agents of the present invention. In the above table columns 1 through 4 indicate the mole percents of the cyclic compounds listed, silver thiocyanate, gold and iodide, respectively. The fifth column gives the access time which is the amount of time required to produce a visible image upon latensification. The sixth column gives the density difference which indicates contrast between the image and background.

The above test results were obtained using relatively small samples of photographic emulsion. When scaled up to production size quantities, it has been found that the optimum concentration of silver thiocyanate is about one-fourth that of the laboratory scale optimum. The increase in sensitization obtained with larger batches is believed to be caused by a number of variables which have not been duplicated in laboratory scale apparatus. For example, the scale up probably changes the average particle size, particle size distribution and ripening conditions caused by differences in agitation and in heating and cooling cycles between large and small batches. Further, it is believed that silver thiocyanate reacts with the surface of the silver halide particles. Accordingly, the surface area available to the silver thiocyanate affects this reaction. Sensitization will depend, therefore, on gel concentration, temperatures and ripening conditions and also on the particle size of the silver halide when the silver thiocyanate is added. The preferred quantity of silver thiocyanate for large scale lots is about 2 mole percent based on the moles of silver in the silver halide grains.

Although specific components and proportions have been described in the above Examples, other suitable materials, as listed above, may be used with similar results. In addition, other materials may be added to the

triazoindolizine, matting agents, etc., may be used in the emulsion layer.

Other modifications and ramifications of the present invention will occur to those skilled in the art upon a reading of the present disclosure. These are intended to be included within the scope of this invention.

#### What is claimed:

1. A photosensitive direct-print light developable emulsion comprising silver halide grains, a binder, iodide and a cyclic compound having the general formula:



50 wherein X is selected from the group consisting of S and Se; and hydrogen and lower alkyl substitution products thereof; said cyclic compound being present in an amount effective to sensitize said emulsion.

2. The emulsion of claim 1 wherein there is included from about 0.01 to about 25 mole percent iodide based on the moles of silver in the silver halide grains.

55 3. The emulsion of claim 1 wherein there is also included from about 0.01 to about 25 percent iodide and from about 0.001 to about 1.0 mole percent gold based on the moles of silver in the silver halide grains.

60 4. The emulsion of claim 1 wherein there is included from about 0.5 to about 9.0 mole percent silver thiocyanate, about 0.4 to about 10 mole percent iodide and about 0.01 to about 0.1 mole percent gold based on the moles of silver in said silver halide grains.

65 5. The emulsion of claim 1 wherein said compound is selected from the group consisting of tetrahydrothiophene-1, 1-dioxide; 2,5-dihydrothiophene-1,1-dioxide;

3-methyltetrahydrothiophene-1,1-dioxide and 3-methyl-2,5-dihydrothiophene-1,1-dioxide.

6. The emulsion of claim 1 wherein said compound is present in an amount of from about 0.02 to about 20 mole percent based on the silver in the silver halide grains.

7. A photosensitive direct-print light developable emulsion comprising silver halide grains, a binder, from about 0.01 to about 25 mole percent iodide, from about 0.001 to about 1.0 mole percent gold, from about 0.5 to about 9.0 mole percent silver thiocyanate, and from about 0.02 to about 20 mole percent of a cyclic compound having the general formula:



wherein X may be S or Se; and hydrogen and lower alkyl substitution products thereof.

8. The emulsion of claim 7 wherein said compound is selected from the group consisting of tetrahydrothiophene-1,1-dioxide; 2,5-dihydrothiophene-1,1-dioxide; 3-methyltetrahydrothiophene-1,1-dioxide and 3-methyl-2,5-dihydrothiophene-1,1-dioxide.

\* \* \* \* \*

UNITED STATES PATENT OFFICE  
CERTIFICATE OF CORRECTION

Patent No. 3,849,146

Dated November 19, 1974

Inventor(s) David W. Walters, Robert E. Heeks, Donald P. Sullivan

It is certified that error appears in the above-identified patent  
and that said Letters Patent are hereby corrected as shown below:

Column 5, Table, Example X, under "access time",  
" > " should read -- < -- .

Signed and sealed this 14th day of January 1975.

(SEAL)

Attest:

McCOY M. GIBSON JR.  
Attesting Officer

C. MARSHALL DANN  
Commissioner of Patents